

(No Model.)

H. AIGNER.

ARTIFICIAL FUEL.

No. 314,097.

Patented Mar. 17, 1885.

Fig. 1



Fig. 2



Fig. 3



Fig. 4



Fig. 5



Witnesses:

E. L. Connolly  
Willibell Powell

Inventor

Hermann Aigner  
By Connolly Bros.  
Attorneys

# UNITED STATES PATENT OFFICE.

HERMANN AIGNER, OF VIENNA, AUSTRIA-HUNGARY.

## ARTIFICIAL FUEL.

SPECIFICATION forming part of Letters Patent No. 314,097, dated March 17, 1885.

Application filed December 8, 1884. (No model.) Patented in Austria-Hungary June 29, 1884, No. 34 and No. 1,079.

*To all whom it may concern:*

Be it known that I, HERMANN AIGNER, a subject of the Emperor of Austria, and a resident of Vienna, in the Empire of Austria, 5 have invented certain new and useful Improvements in Artificial Fuel, of which the following is a specification.

According to the present improvements a mixture of coal-tar pitch and vegetable fiber is molded into perforated blocks or bricks, which are then coked, and finally again pressed and perforated.

With reference to the accompanying drawings, Figures 1 and 2 are views, and Figs. 3 and 4 sections, of fuel-bricks in natural size and manufactured according to the present invention.

The process of executing the present improvements is as follows: One hundred pounds 20 of ordinary coal-tar pitch are successively melted in a boiler, and then five hundred pounds of vegetable fiber are intimately mixed with the melted pitch. As vegetable fiber we preferably employ waste cotton and wood, or 25 any other suitable organic fibrous material which on combustion evolves only hydrocarbons and leaves little or no ashes. The thorough mixing of the materials may be effected by any mechanical agitator, and is continued 30 until the mass has assumed a dough-like consistency. The mixture is removed from the boiler and is spread over heated stone flags, and is then molded into pieces of 2 by 2 by 4

inches and perforated. These perforated bricks are then subjected to dry distillation or 35 coking in the same way as coals in manufacturing coal-gas. This coking is effected, as indicated by Fig. 5, in a wire-gauze cylinder, *a*, into which the perforated blocks arranged on the rod *b* are inserted. The cylinder *a* is 40 put into a retort, *c*, provided with gas-escape pipes *c'*. A number of such retorts *c* are arranged in a furnace of the same kind as those used in ordinary works for manufacturing ordinary coal-gas. The blocks thus coked are 45 again molded while warm, so that they assume the perforated and beveled shape shown in the drawings.

The hole shown in the drawings forms a passage for the flame, and largely contributes to 50 increasing the heat of combustion.

I claim—

The described method of manufacturing artificial fuel, consisting in forming perforated blocks of a mixture, substantially as described, 55 of coal-tar pitch and vegetable fiber, subsequently coking such blocks, and in finally pressing the same into the perforated beveled shape, essentially as described, and shown in the drawings.

In testimony whereof I have affixed my signature in presence of two witnesses.

HERMANN AIGNER.

Witnesses:

C. O. PAGET,  
E. G. F. ROELLER.